

A. F. SHORE.  
CASE HARDENED STEEL.  
APPLICATION FILED APR. 5, 1913.

1,072,661.

Patented Sept. 9, 1913.

Fig. 1



Fig. 2



Fig. 3



Fig. 4



Fig. 5



Fig. 6



Fig. 7



Witnesses:

Louis Smith Jr.  
Maxwell C. Robson

Inventor  
A. F. Shore  
By his Attorney  
Head & Hoffmann

# UNITED STATES PATENT OFFICE.

ALBERT F. SHORE, OF NEW YORK, N. Y.

## CASE-HARDENED STEEL.

1,072,661.

Specification of Letters Patent.

Patented Sept. 9, 1913.

Application filed April 5, 1913. Serial No. 759,009.

*To all whom it may concern:*

Be it known that I, ALBERT F. SHORE, a citizen of the United States, residing at New York, in the county of New York and State 5 of New York, have invented certain new and useful Improvements in Case-Hardened Steel, of which the following is a full, clear, and exact specification.

This invention relates to case-hardened 10 steel, and the object of the invention is the production of a structure in steel suitable for armor-plates, large guns, projectiles, or machine elements or parts thereof, and composed of two or more layers or sections of 15 different degrees of hardness and arranged so as to interlock to prevent peeling or flaking.

In my pending application Serial Number 627,747, I have described and claimed the 20 process for case-hardening steel, the result of which process is the subject of the present application.

In the drawing forming part of this specification, I have illustrated steel plates characterized by having two layers of different 25 degrees of hardness and interlocked or so arranged that there is an irregular plane of separation between the layers, and the novel features of the product are pointed out in 30 the claim.

Figure 1 is a cross-sectional view of a steel plate embodying my invention. Figs. 2, 3, 4, and 5 illustrate modified forms or arrangements of the interlocking layers, and 35 Figs. 6 and 7 illustrate two different means used for carrying out the process for producing the steel plates shown in the other figures.

The process is described in detail in the 40 pending application referred to and embodies the partial covering of the steel plate 6 by a suitable carbon-resisting agent, such as cement for instance, which may be put on the plate in the preferred form, as shown at 45 7, which leaves uncovered and therefore unprotected the portions 8 of the plate. Or, as shown in Fig. 7, the covering may be in the form of individual disks 9. Thereafter, the plate is carburized to the desired depth at 50 the portions 8.

The result of the process is illustrated in

Fig. 1, in which 11 represent the carburized portions of the plate and 13 represents the softer backing. 12 represent the protected or covered areas on the plate, where the material has also been carburized but to a less degree than at 11, and, due to the peculiar action of carbon infusion which penetrates laterally under the covering as well as going straight down but to a less degree. Thus 60 there are formed two adjacent layers or sections, namely 11 and 13, with no straight plane of separation between them, but each of them having portions 14 and 15 which interlock or invade the adjacent section or 65 layer, and whereby peeling or flaking is prevented and crushing strains or blows localized.

By making the protective covering small or narrow, as shown in dotted lines in Fig. 70 2 at 16, the interlocking portion 17 of the layer 13 is made quite small and pointed.

Fig. 3 illustrates the results obtained when the covering 18 is quite broad and only semi-resistant to carbon. In this instance 75 the interlocking portion 19 is large. The semi-resistant may in this instance consist of cement as above, but in a more porous state.

Fig. 4 shows the results obtained by employing two narrow coverings 20, close to one another. In this instance the interlocking portion comprises two adjacent pointed portions 21.

Fig. 5 shows a covering composed of partial carbon-resisting material 22 as a semi-porous cement in the middle and absolute carbon-resisting material 23 on both sides, and whereby the interlocking portion 24 becomes large with an irregular line of separation between it and the layer 11.

It will be apparent that in each of the instances illustrated I have produced a unitary steel plate composed of two sections or layers of different degrees of hardness having 95 an irregular plane of separation between them and whereby each section is formed with interlocking portions extending beyond or inside the area of the adjacent section.

I claim:

As a new article of manufacture, a unitary steel plate consisting of a single integral

piece of material comprising a body portion and a face portion, said face portion being of greater hardness and less thickness than the said body portion, both of said portions 5 of the single piece of material having regularly formed interlocking spaced portions extending into each other.

In testimony whereof, I affix my signature, in presence of two witnesses,

**ALBERT F. SHORE.**

Witnesses:

**MARTHA W. SHAW,  
CHAS. BELMAR.**